

# United States Patent

Mitchell, Jr.

[15] 3,639,957

[45] Feb. 8, 1972

[54] **PAPER MANUFACTURING ROLL CONSTRUCTION AND PROCESS**

2,730,770 1/1956 Higginbotham et al.....29/120 X  
2,804,678 9/1957 Rockoff .....29/121 R  
3,460,222 8/1969 Mitchell.....29/120

[72] Inventor: Paul J. Mitchell, Jr., Griffin, Ga.

Primary Examiner—Alfred R. Guest  
Attorney—Morse, Altman & Oates

[73] Assignee: SW Industries, Inc., Newton, Mass.

[22] Filed: June 6, 1969

[21] Appl. No.: 831,161

**Related U.S. Application Data**

[63] Continuation-in-part of Ser. No. 606,412, Dec. 30, 1966, Pat. No. 3,460,222.

[52] U.S. Cl.....29/120

[51] Int. Cl.....B21b 31/08

[58] Field of Search .....29/120, 125, 132

[56]

**References Cited**

**UNITED STATES PATENTS**

2,497,696 2/1950 Smith.....29/120 X

[57] **ABSTRACT**

In a paper making machine, following casting of the aqueous pulp suspension onto a moving web and partial drainage of water therefrom to form a wet sheet, water is pressed from the wet sheet by rolls that are characterized by a covering composed of a butadiene acrylonitrile elastomer and a dispersion of hydrophobic fiber strands penetrating through the outer surface of the elastomer. Such rolls have superior release characteristics with respect to the wet sheet.

2 Claims, 2 Drawing Figures



PATENTED FEB 8 1972

3,639,957



FIG. 1



FIG. 2

INVENTOR

BY *Paul J. Mitchell, Jr.*  
*Morse, Altman & Oates*

ATTORNEYS

## PAPER MANUFACTURING ROLL CONSTRUCTION AND PROCESS

### CROSS-REFERENCE TO RELATED APPLICATIONS

This is a continuation-in-part of Ser. No. 606,412, filed Dec. 30, 1966, in the name of P. J. Mitchell, Jr., for PAPER MANUFACTURING ROLL CONSTRUCTIONS AND PROCESSES, now U.S. Pat. No. 3,460,222 issued to the assignee of this application.

### SUMMARY OF THE DISCLOSURE

The present invention relates to papermaking machines and processes and, more particularly, to enhancement of the release characteristics of rolls in contact with the advancing wet sheet following casting of the aqueous pulp suspension in any of the several different types of paper forming processes. In a typical papermaking process, a dilute aqueous slurry of cellulose fibers, which have been produced by grinding wood pulp or the like, first is cast on an endless wire screen through which water is drained, next is advanced into an endless felt, with which it passes between a series of so-called press rolls that squeeze and withdraw water therefrom, next is advanced by itself between a series of press rolls and then is advanced over heating drying cylinders. Difficulties have been encountered as a result of a tendency by fibers of the wet sheet to adhere to the press rolls with which they come in contact.

The primary object of the present invention is to provide improved release characteristics in the elastomeric cover of a press roll for paper sheet formation by the addition of fine fiber strands, ends of which penetrate and protrude through the finished, ground outer surface of the rubber cover. In accordance with the present invention, the elastomeric cover is composed of butadiene acrylonitrile. It is believed that, when the fibers are hydrophobic, the surface tension of a water film on the rubber cover surface is interrupted in such a way as to decrease adhesion of the wet paper filaments to the rubber cover surface as a whole. Other objects of the present invention will in part be obvious and will in part appear hereinafter.

### DESCRIPTION OF THE DRAWINGS

The invention accordingly comprises the devices and processes possessing the particular components, steps and interrelationships, which are exemplified in the following detailed disclosure, the scope of which will be indicated in the appended claims. For a fuller understanding of the nature and objects of the present invention, reference is to be had to the following description taken in connection with the accompanying drawings, wherein:

FIG. 1 is a distorted cross-sectional, schematic view of a portion of a papermaking machine embodying the present invention; and

FIG. 2 is an exaggerated cross-sectional, broken-away detail view of one of the rolls of the construction of FIG. 1.

### SPECIFIC DISCLOSURE

In a papermaking process involving the present invention, the initial wet sheet 10, is formed by casting a dilute aqueous slurry of cellulose fibers onto an endless wire screen 11, as is shown in FIG. 1. In accordance with the present invention a so-called lumbbreaker roll 14, which is a press roll embodying the present invention, serves to contact the advancing paper sheet in such a way as to flatten uneven agglomerations of fibers in various portions of the advancing sheet. The sheet next advances onto an endless felt 12. The wet sheet and the felt advance into engagement between a series of press rolls, two of which are shown at 16, 18, after the sheet is separated from screen 11 at 15. Then the wet sheet advances between the nips of a series of press rolls, two of which are shown at 20, 22. When advancing over wire screen 11, on felt 12 and in contact with the various press rolls, generally the moisture content by total weight of the sheet is in excess of 35 percent. The rolls in direct contact with the wet sheet, during this time,

are characterized by exceptional release properties in accordance with the present invention. It will be understood that such direct contact rolls may be above and/or below the advancing paper sheet.

As shown in FIG. 2, each of press rolls 14, 16, 20 and/or 22 is shown as having a metal core 24 and an elastomeric veneer 26. The metal core, for example, is in the form of a solid or hollow cylinder composed of metal such as steel or cast iron, or other dimensionally stable material. The veneer contains a matrix of an elastomer 28 and dispersed, randomly distributed fiber strands 30. For best results in accordance with the present invention, the elastomer is composed of butadiene acrylonitrile. Preferably, the fiber strands are composed of a hydrophobic synthetic polymer, and, most advantageously, are selected from the class consisting of polyesters, polyamides and acrylics. Best results have been achieved with linear polyamides such as polyhexamethylene adipamide. For present purposes, the term hydrophobic is applied to a material having a regain of moisture from a bone dry condition of less than 5 percent based on original bone dry weight in an atmosphere having 65 percent relative humidity at 75 percent F. Preferably, by total weight of the combination, the strands range from 0.5 to 10.0 percent and the elastomeric matrix ranges from 99.5 to 90 percent. For best results, the strands range from one-half to 5 denier and from one sixty-fourth to 2 inches long. Preferably the final composition ranges from 20 to 200 plastometer,  $\frac{1}{8}$ -inch ball, Pusey and Jones.

### EXAMPLE I

A press roll of the foregoing type was produced as follows. Polyhexamethylene adipamide strands, 1 $\frac{1}{2}$  denier and 1 $\frac{1}{2}$  inches long, were uniformly dispersed into a mass of uncured butadiene acrylonitrile elastomeric matrix. The resulting dispersion of strands in the matrix was such that, by total weight, the strands were approximately 5 percent and the elastomeric composition was approximately 95 percent. The elastomeric composition was formulated in accordance with typical practice to give a hardness of 35 plastometer,  $\frac{1}{8}$ -inch ball, Pusey and Jones. An iron core, 34 inches in diameter by 184 inches in length, was cleaned and roughened by grit blasting and coated with cement in accordance with well established roll covering techniques. The foregoing formulation was applied in a 1 inch thickness onto the iron core and cured, finished and ground in accordance with well established roll manufacturing techniques. Examination revealed that the ends of the strands penetrated through the ground surface of the chloroprene roll cover. This ground surface was characterized by exceptional release characteristics with respect to wet paper sheet in contact therewith.

### EXAMPLE II

The foregoing example is repeated with 50, 75 and 100 plastometer,  $\frac{1}{8}$ -inch ball, Pusey and Jones, with similarly excellent results.

### OPERATION AND CONCLUSION

The superior release characteristics of the rolls illustrated above are believed to be based, at least in part, on the effect of the free ends of the fiber shreds on the surface tension of a film of water on the roll. These free ends interrupt the uniform wetting of the roll by the wet paper sheet and, thereby, interrupt the uniformity of the surface tension of the layer of water that otherwise would exist on the roll cover. The result is that cellulose fibers from the wet paper sheet, which are swollen with moisture, have a greatly decreased tendency to adhere to the surface of the roll.

Since certain changes may be made in the foregoing disclosure without departing from the scope of the invention involved, it is intended that all matter shown in the accompanying drawing and described in the foregoing specification be interpreted in an illustrative and not in a limiting sense.

I claim:

1. A roll for use in a paper making machine, said roll comprising a cylindrical core and a veneer, said veneer having an elastomeric matrix and fiber strands dispersed therein, free ends of said strands penetrating and protruding through the outer surface of said elastomeric matrix, said strands being composed of a hydrophobic synthetic polymer selected from the class consisting of polyesters, polyamides and acrylics, said matrix being composed of butadiene acrylonitrile.

2. The roll of claim 1 wherein said strands are composed of a linear polyamide, being approximately within the ranges of one-half to 5 denier in diameter and one sixty-fourth to 2 inches in length, said strands by total weight of said veneer ranging approximately from 0.5 to 10 percent and said elastomeric matrix by total weight of said veneer ranging approximately from 99.5 to 90 percent.

\* \* \* \* \*

10

15

20

25

30

35

40

45

50

55

60

65

70

75